

J. KIRBY.

METHOD OF WELDING A PROTECTIVE COVERING OF COPPER TO AN IRON OR STEEL BODY.  
APPLICATION FILED DEC. 8, 1915.

1,211,715.

Patented Jan. 9, 1917.

Fig. 1.



Fig. 2.



Inventor:  
John Kirby  
By Max H. Solovitz  
Attorney.

# UNITED STATES PATENT OFFICE.

JOHN KIRBY, OF PITTSBURGH, PENNSYLVANIA.

## METHOD OF WELDING A PROTECTIVE COVERING OF COPPER TO AN IRON OR STEEL BODY.

1,211,715.

Specification of Letters Patent.

Patented Jan. 9, 1917.

Application filed December 8, 1915. Serial No. 65,665.

*To all whom it may concern:*

Be it known that I, JOHN KIRBY, a citizen of the United States, residing at Pittsburgh, in the county of Allegheny and 5 State of Pennsylvania, have invented certain new and useful Improvements in Methods of Welding a Protective Covering of Copper to an Iron or Steel Body, of which the following is a specification.

10 This invention relates to a method of welding a protective covering of copper to an iron or steel body and has for its object to provide a method, in a manner as hereinafter set forth, whereby copper sheets, 15 plates, cylinders, sleeves, jackets, etc., can be welded to the exposed surface or surfaces of an iron or steel body so as to prevent such surface or surfaces from corroding or rusting from atmospheric action, which 20 otherwise would be the case when the exposed surface or surfaces is or are subjected to the action of the atmosphere. The rusting or corroding of the exposed surface or 25 surfaces of the iron or steel body greatly impairs the commercial usefulness of such body as is obvious.

A further object of the invention is to provide a method, in a manner as herein-after set forth, for the purpose of setting up 30 a copper surface for iron or steel to protect the latter against corrosion by atmospheric influences or against any chemical action to which copper is immune.

Briefly described the method consists in 35 the setting up of a copper covering, such as a copper plate, sheet, cylinder, etc., within a mold and then running or pouring into the mold against the inner face of the covering molten iron or steel, at as low a tempera- 40 ture as is consistent with a fluid state. The heat of the metal will attack the inner face of the covering sufficiently to soften said inner face and the copper in such condition will readily unite with the iron or steel dur- 45 ing the solidification of the latter and have all the characteristics and withstand all the usual tests of a true weld.

As illustrating, by way of example, a pair 50 of molds for carrying the method into effect reference will be had to the accompanying drawing in which—

Figure 1 is an elevation of a mold em- 55 ployed when covering the ends or sides of an iron or steel body. Fig. 2 is an elevation

of a mold employed when forming a copper 55 covered billet from which wire is drawn.

Referring to Fig. 1 of the drawing 1 de- 60 notes a rectangular mold provided with a gate 2 and 3 denotes the copper plates which form the covering for the sides of the iron 65 or steel body.

Referring to Fig. 2 of the drawing 4 de- 70 notes a cylindrical mold having a gate 5 and 6 denotes a copper shell or cylinder which forms the covering for the billet from 75 which wire is drawn.

An example of carrying the method into 80 effect when it is desired to cover the ends of the sides, of an iron or steel body is as follows:—A suitable chilled mold is set up 85 of the shape desired and within the molding cavity, at opposite sides of the wall thereof are positioned the copper sheets or plates. Molten steel or iron, at as low a tempera- 90 ture as is consistent with a fluid state of the metal, is poured into the molding cavity, the temperature of the metal is from 2400 degrees to 2600 degrees Fahr. The molten metal is supplied to the molding cavity be- 95 tween the copper plates, in such a manner that the inflowing metal flows gently against the inner faces of the copper plates, imparting to them a degree of heat sufficient to soften the said inner face without however reducing the copper to a molten state or cause the plates to lose their original shape. In this softened condition the copper will readily and firmly unite with the metal and provide a bond having all the characteristics and withstanding all the usual tests 95 of a true weld, moreover the temperature of the metal at the moment of its contact with the copper plates precludes oxidization of the surfaces of the metal and at such point preventing the formation of foreign oxides which would by their presence destroy the weld.

If desired during the welding operation the mold can have the walls thereof cooled, for example by employing a water jacket, 100 under such conditions preventing that surface of the copper plate opposing the wall and which is not engaged by the molten metal from becoming heated.

If a large ingot or billet is to be molded 105 and to prevent the heat of the metal having effect upon the copper so as to melt it, protecting metallic plates of the same material

as the ingot or billet can be arranged within the mold and spaced from the copper. Said protecting plates would have openings or gates to allow the metal to flow between the 5 plates and the copper and by such an arrangement such metallic plates would protect the copper. The metallic plates would be of the same length and height as the billet to be formed and would be cast therewith.

10 The employment of such plates is to prevent the heat of the molten metal attacking the copper to melt the same. When the mold has been filled to its capacity its combined contents are allowed to solidify and the billet 15 thus formed will be ready for the rolls.

When forming a copper covered billet from which wire is drawn, the molten metal is poured into a copper cylinder, the latter being positioned or clamped within a mold 20 and if desired the outer face of the cylinder can be cooled so that the heat from the molten metal when poured into the cylinder will not cause the latter to lose its original shape. After the cylinder has been filled 25 with the metal, the latter is allowed to solidify which provides for a perfect weld between the copper and metal and overcomes the necessity of sealing the ends of the billet when drawing the wire.

30 What I claim is:—

1. A method of welding a protective covering of copper to an iron or steel body comprising the softening of the inner face of a solid copper body by bringing into 35 gradual contact with said inner face the metal to be protected when in a molten state and at a temperature from 2400 degrees F. to 2600 degrees F., and then allowing the molten metal to cool to cause the solidifica-

tion of such metal with the copper thereby 40 setting up a perfect weld between the copper and the solidified metal.

2. A method of welding a protective covering of copper to an iron or steel body comprising the positioning of the covering 45 formed of a solid copper body within the molding cavity of the mold, then supplying the metal to be protected at a temperature from 2400 degrees to 2600 degrees F. to the molding cavity of the mold to gradually contact with the inner face of said copper body to soften said inner face, and then allowing the molten metal to cool to cause the solidification of such metal with the copper thereby 50 providing a perfect weld between the copper and the solidified metal.

3. A method of welding a protective covering of copper to an iron or steel body comprising the positioning of the covering formed of a solid copper body within the 60 molding cavity of the mold, so that the outer face of the copper body will oppose the wall of the molding cavity, then supplying the metal to be protected at a temperature from 2400 degrees to 2600 degrees F. to the molding cavity of the mold to gradually contact with the inner face of said copper body to 65 soften said inner face, and then allowing the molten metal to cool to cause the solidification of such metal with the copper thereby 70 providing a perfect weld between the copper and the solidified metal.

In testimony whereof I affix my signature in the presence of two witnesses.

JOHN KIRBY.

Witnesses:

NICHOLAS L. BOGAN,  
A. L. SROLOVITZ.